

106-18.12

SR

OR 2,553,781

## UNITED STATES PATENT OFFICE

2,553,781

## FLAME RESISTANT CELLULOSE FIBROUS MATERIALS AND METHOD OF MAKING SAME

Ralph R. Oliver, Lockport, N. Y., assignor to Lockport Cotton Batting Co., Lockport, N. Y.

No Drawing. Application April 14, 1950,  
Serial No. 156,050

2 Claims. (Cl. 117—137)

1

This invention relates to improvements in fibrous or cellulosic materials of vegetable origin, and to methods of making the same flame or flash resistant.

This is a continuation-in-part of my pending application No. 735,022, filed March 15, 1947, which in turn was a continuation in part of my copending application Serial No. 434,917, filed March 16, 1942, and now abandoned.

Heretofore in treating organic vegetable fibers for this purpose, for example, according to my Patent No. 2,135,695 of January 2, 1940, the cotton or other fibers have been kier-boiled with caustic soda and then bleached, washed and at least partly dried. The vegetable fibers were then put through a washer containing a solution of borax and boric acid. Because the vegetable fibers are absorbent after this boiling and bleaching operation, the borax and boric acid are readily absorbed thereby. The excess solution was then removed and the fibers dried.

One of the objects of this invention is to provide raw and unbleached cellulosic fibers of vegetable origin which are flame and flash resistant. Another object is to provide an improved and simplified method of rendering organic vegetable fibers fire-resistant and in which method the steps of kier boiling and rinsing the fibrous material may be dispensed with. Another object of this invention is to treat raw fibers of vegetable origin in a single step process to make the same flame and fire-resistant without interfering with the free flexibility of the fibers, so that the fibers can be worked on machines without substantial loss due to breakage of the fibers, which process will be relatively simple, inexpensive, efficient and safe. Other objects and advantages of this invention will appear from the following description and claims.

In accordance with my improved process, the loose, unspun and unwoven raw vegetable fibers are treated in a bath containing a flame and flash resistant agent, such as borax and boric acid, and a surface active agent. Any suitable or desired anionic or non-ionic surface active or wetting agent may be employed, many agents of this type being now available on the market. For example, any of the following materials may be employed as surface active agents:

Alkyl aryl sulphonate  
Diocetyl ester of sodium sulfosuccinic acid  
Polymerized ethylene oxide condensate  
Sulfated fatty alcohol  
Alkali soap of naphthenic acid  
Quaternary ammonium salts

2

The reason for using surface active agents is to induce and increase the penetration of the solution of the chemical or chemicals used into the fibers and to wet the surface of the fibers, to

produce the desired effect, after drying the fibrous material, of rendering the material flame and flash resistant. Raw fibers of vegetable origin are usually coated or impregnated with oily or waxy substances which prevent the penetration of water into the fibers and which prevent the adhesion of water on the fibers, unless the fibers are first subjected to a kier boiling or saponifying operation in which the oily and wax-like coating materials of the fibers are dissolved or removed from the fibers. I have found, however, that by use of anionic or non-ionic surface active agents, the water in which the borax and boric acid are dissolved will readily penetrate the fibers and will adhere to the surfaces

20 thereof.

The borax and boric acid are present in the bath or solution in the desired quantities to deposit sufficient of these materials on the fibers to produce the desired flame resistant properties 25 and to produce a solution having a pH between 7 and 8. The pH should not be below 7, since a breakdown or deterioration of the fibers results if the solution is on the acid side.

I have found that in the carrying out of this process a careful control of the temperature of the solution containing the borax, boric acid and surface active agent should be maintained so that the best results are obtained. For this reason, the temperature of the bath or solution is 30 preferably approximately from 130° to 212° F., 130° to 140° F. being the best average operating temperature. If the temperature of the bath is materially below 130 F., the optimum results are not obtained for the reason that the solution does not thoroughly penetrate into the fibers so that insufficient borax and boric acid are deposited within the fibers by capillary action and absorption. Furthermore, borax and boric acid are more readily soluble in warm water than in cold water, and it is desirable to have the bath 35 as concentrated as possible to deposit the maximum quantity of borax and boric acid on and in the fibers, and if the solution drops below 130° F., some of these ingredients crystallize out of the solution. If the temperature is materially over 150° F., the fibers tend to become somewhat more brittle due to breakdown of the cellulosic material. This is particularly noticeable during the mechanical treatment of the cotton, such 40 as carding and garnetting.

106/15F

106/163R

106/166C

In the use of this process on vegetable fibers, such for example as cotton, the material from the bales is first fluffed up in any usual or suitable manner such as heretofore commonly employed, and the fibrous material is then discharged into a tank containing the bath and is kept submerged in the bath while passing from one end of the tank to the other. At the other end of the tank the vegetable fibers are withdrawn from the bath and excess solution is pressed out of the material. This may, for example, be accomplished by passing the material between rollers which squeeze out excess solution from the fibrous material, so that the amount of solution left in and on the fibrous material is about from 30% to 50% of the weight of the fibrous material. It is desirable to leave a certain amount of this solution on the outer surfaces of the fibers so that when the fibers are dried, the required amount of borax and boric acid is left on the surfaces of the fibers as well as in the interior thereof. The cotton or other fibrous material may then be dried in any suitable or desired manner, for example in a raw stock drier, such as commonly used in the treatment of cotton. This drier removes the water from the fibrous material and leaves the borax and boric acid in and on the fibers, and thus makes the same resistant to flame and fire, without, however, changing the flexibility of the fibers and without making them brittle. The drying is preferably carried on until about 8% to 10% of moisture remains in the material.

As an example of the treatment of cotton and other vegetable fibers in accordance with this invention to render them flame resistant without subjecting the fibers to a kier boiling process, the flame proofing ingredients are dissolved in water in the proportion of one to two pounds per gallon of water, these ingredients including approximately two parts by weight of borax to one part of boric acid. The resulting solution will then have a pH of approximately from 7 to 8. To this solution is added approximately from one-tenth to one-half of one percent by weight of the solution of a suitable surface active agent, which percentage may be varied according to mill conditions and according to variables that occur in all raw water. The final solution is raised to a temperature between 130° F. and 212° F., about 130° F. to 140° F. being preferred, and the raw cotton or other vegetable fibers are then immersed in this solution until the fibrous material is completely wetted out. The surface active agent greatly increases the penetrating action of the solution so that the same fills the canals of the fibers and penetrates the fiber walls or cells. In such a bath, the raw, previously untreated fibers very rapidly sink and become fully impregnated and saturated with the solution. Generally after the cellulosic material has been immersed in the solution for about two minutes, the solution will have fully penetrated the fibers. The fibrous material is then withdrawn from the solution and pressed to remove excess solution, leaving from 30% to 50% of solution by weight of the fibrous material thereon, and dried as already described.

After the fibers have been dried, the weight of the same is increased about 12% to 15%, due to the absorption and incrustation of the flame-

proofing substances in and on the fibers, and the fibers are not brittle and may be worked in any of the usual machines, such as carding and garnetting machines, in which the fibers are formed into resilient batts suitable for house and building insulation, or for other purposes. It has also been found that fibers treated in accordance with my process are stronger and better adapted for heat insulation than fibers which have been kier boiled. Heretofore in processes for making cotton fire resistant, a certain percentage of the fibers has been lost during the flame-proofing of the same because preliminary kier boiling made these fibers brittle, but with my improved treatment, in which no kier boiling or saponification is necessary or desirable, the loss of fibers is substantially avoided. The term "raw" as herein applied to vegetable fibers includes not only the fibers as they come from the plants, but also gray stock, which has not been chemically treated or kier boiled.

It will be understood that various changes in the details, materials and conditions, which have been herein above described in order to explain the nature of the invention may be made by those skilled in the art within the principle and scope of the invention, as expressed in the appended claims.

I claim as my invention:

1. A method of treating loose, raw, cellulosic fibers to render the same flame and fire resistant without substantially changing the flexibility of the fibers and wherein the fireproofing composition is deposited on and in the fibers, which method comprises subjecting the raw fibers to an aqueous solution maintained at a temperature between 130° F. and 150° F. and at a pH of approximately between 7 and 8, said solution containing borax, boric acid and a compatible surface active agent, the borax being present in the proportion of the approximately 1 pound per gallon of water, the boric acid being present in an amount of approximately  $\frac{1}{2}$  pounds per gallon of water and the surface active agent being present in an amount of approximately  $\frac{1}{10}$  to  $\frac{1}{2}$  percent by weight of the solution, heating the solution, and maintaining it at a temperature within the range indicated, leaving the fibrous material in said solution for at least two minutes, removing the material from said solution, removing solution from said material until the amount of solution adhering to the material is equal to approximately 30% to 50% by weight of the material and then drying the material, whereby the amount of flame and fireproofing composition deposited on and in the fibers is from about 10% to 15% by weight of the fibrous material.

2. A flame and flash resistant, loose, raw cellulosic material having substantially the properties of the product resulting from treatment by the process of claim 1.

RALPH R. OLIVER.

#### REFERENCES CITED

65 The following references are of record in the file of this patent:

#### UNITED STATES PATENTS

| Number    | Name          | Date         |
|-----------|---------------|--------------|
| 2,178,625 | Clayton _____ | Nov. 7, 1939 |
| 2,185,695 | Oliver _____  | Jan. 2, 1940 |